

## UNITED STATES PATENT OFFICE

JOHN WESLEY MARDEN AND HARVEY CLAYTON RENTSCHLER, OF EAST ORANGE, NEW JERSEY, ASSIGNEES TO WESTINGHOUSE LAMP COMPANY, A CORPORATION OF PENNSYLVANIA

## COMPOSITE BODY AND METHOD OF PRODUCING THE SAME

No Drawing.

Application filed August 1, 1921. Serial No. 489,108.

This invention relates to composite bodies and to processes for the production of the same and, more particularly, it pertains to a process for the production of composite bodies of refractory metals and to the articles produced thereby.

It is necessary or advantageous in many arts to employ, in lieu of a single homogeneous material, composite bodies consisting of consolidated materials having different properties. Conditions making such composite bodies desirable arise, for instance, when a small amount of comparatively expensive material, used in combination with a cheaper material, will serve the same purpose as a body or article consisting entirely of the former. As an example of such combination, the coating of a common metal with platinum for use as electrodes in the electro

chemical arts may be cited.

Other circumstances requiring a composite body arise when a material having valuable properties can, only with difficulty, be fabricated singly to adapt it for practical use but may be more readily worked as one of the elements of a combination. An example of such character is present when it is desired to utilize metallic thorium as electron-emission material in electrical devices, such as vacuum tubes used in wireless apparatus, hot-cathode rectifiers of the Rectigon type and X-ray tubes, all of which require a heated filament and preferably one having high electron emissivity at temperatures not incompatible with a long-burning life. For such purposes, the thorium should be drawn into wire form to adapt it to be heated by the electric current. It has been found possible by employing the process hereinafter described, to readily produce a composite wire comprising a base material, such as molybdenum, coated with thorium, which, as an electron-emission material, is as valuable as a wire consisting entirely of metallic thorium.

In other circumstances a composite body is superior to a homogeneous body. For example, an X-ray target at which X-rays are generated preferably consists of a refractory metal of high atomic weight and another metal of high heat-dissipating capacity, the

former being necessary for the generation of powerful X-rays and the latter so that the heat generated by electronic bombardment of the target may be dissipated rapidly enough to prevent the temperature from rising to the melting point of the material of which the target is composed. Such composite target may consist of a metal of high atomic weight, such as thorium, consolidated with a body having a high heat-dissipating capacity, such as copper, chromium or other metal. The composite bodies for such purposes may be very conveniently prepared by the process of the present invention.

It is, therefore, an object of the present invention to provide a process for the production of composite bodies and, more particularly, for the production of such bodies consisting of at least one refractory metal.

Another object of our present invention is the provision of a composite body consisting, at least in part, of a metal of high electron emissivity.

A further object of the invention is the provision of composite bodies which shall be valuable in increasing the efficiency and the burning life of electric devices, such as incandescent electric lamps and the like.

Other objects of the present invention will be apparent from a reading of the following specification.

In order to secure the advantages of composite bodies, well-known methods such as rolling, drawing and electrolytic deposition have been employed. These methods have often been successful when the materials to be united were malleable, ductile, or did not easily combine chemically with other elements. When, however, the materials sought to be combined did not possess the requisite properties for such methods of fabrication, combinations of certain materials having valuable properties were not available. For example, the combination of a non-ductile metal, such as zirconium, could not be drawn in connection with another material as a base. Up to the present time it has been found that certain refractory metals cannot be united solely by means of heat when in contact with each other. For example, an un-

successful attempt was made to coat a tungsten wire with thorium by surrounding the former with a quantity of thorium powder. The two metals, in contact, were heated in a high vacuum to a temperature which would be thought sufficient to cause a union of the two metals. The resultant product, however, when tested for electron emissivity did not give results characteristic of thorium, 10 showing that, if a small quantity of the latter metal did adhere to the tungsten, it very probably was left in such physical condition that it was quickly oxidized when exposed to the air.

15 Other experiments conducted by us have shown that compounds of certain metals cannot be made to form a composite body with another material by applying a compound of the metal to another material as a base, 20 attempting to reduce the metallic compound and subjecting the materials to a heat treatment with a view to effecting a union between the reduced metal and the base material.

25 That part of our present invention which relates to the method of producing composite bodies is particularly valuable for the utilization of those metals which have such a strong chemical affinity for other elements 30 that they should preferably be worked, in combination with another material, in a very high vacuum in order to obtain them in a dense, coherent and adherent mass, and it is still more valuable when dealing with such 35 metals having a high melting point and also in combining with other material metals which, in addition to possessing a strong chemical affinity and a refractory nature, are also difficultly workable by such processes as rolling, swaging, drawing, etc.

40 We have found that composite bodies of certain materials, especially those consisting, in part at least, of one or more metals of comparatively high electron emissivity, 45 serve excellently as an electron-emitting body in electrical devices requiring such bodies, as, for example, vacuum tubes used in wireless apparatus, hot-cathode rectifiers of the Rectigon type, and X-ray tubes. 50 Thorium, zirconium, titanium, uranium and vanadium are examples of metals which can be used to advantage as electron-emission material, especially when forming part of a composite body. The present invention supplies a very satisfactory method of producing composite bodies, utilizing one or more of such metals.

55 We have also utilized the present invention for producing composite bodies of refractory materials suitable for use as filaments in incandescent lamps. In this case, a base material may be coated by any suitable method with a metal or mixture of metals or alloys having desirable properties such, 60 for example, as selective light emissivity.

Another part of our invention consists in the discovery that metals having certain properties are valuable as agents for purifying other materials and for removing or converting from the active phase, materials which act deleteriously under certain circumstances, such as gases or vapors in vacuum and gas filled tubes which employ an incandescent body. Metals, such as zirconium, thorium, uranium, titanium, chromium, metals of the rare earths, aluminum and magnesium, which have a strong chemical affinity for many elements are valuable for purposes of purification. When employed in electrical devices containing an incandescent body, as, 70 for example, a metal-filament incandescent lamp, such metals are especially valuable in removing deleterious gases, such as oxygen, and vapors, such as that of water, which quickly damage incandescent bodies. Water vapor is particularly injurious, inasmuch as the interaction between water vapor and the incandescent filament is a cyclic process, the first step in which is the decomposition of 75 the water vapor by the filament, resulting in the formation of a metallic oxide and free hydrogen. The oxides of many metals, being volatile at the high temperature at 80 which the filament is operated, are thereby vaporized and are subsequently reduced by the hydrogen to produce the original quantity of water vapor and the metal of which the filament consists. The water vapor, being 85 thus renewed again reacts with the incandescent filament, and the cycle described is 90 continuously repeated until the filament 95 burns out.

It will thus be seen that, in order to eliminate water vapor and harmful gases from such devices, metals such as zirconium, 100 thorium, uranium, titanium, chromium, metals of the rare earths, aluminum and magnesium or a combination of two or more 105 of the same, which react with them to form stable compounds therewith and especially 110 those which form compounds not reducible by hydrogen, are effective in maintaining the efficiency and prolonging the burning life of such devices. In the lamp-making art, materials which perform such functions 115 are known as clean-up agents and hereinafter will be referred to as such in referring to incandescent lamps and similar devices.

120 Various methods may be employed for introducing metallic clean-up agents into incandescent lamps and similar devices but a very convenient method is found to be the placement of the clean-up agent on the filament to form a composite body. Preferably, after the lamp has been exhausted and sealed 125 to the atmosphere, the filament is then, for the first time, lighted to incandescence and the clean-up agent is thus activated, that is, made to combine with the residual gases and 130 vapors. Part of the clean-up agent may be

vaporized from the filament, if desired, and the residue permitted to remain on the filament in case of certain metals.

Up to the present time, we have found it best for producing composite bodies consisting, for example, of two materials, to have one of them in the form of particles or in a pulverulent condition, while the material with which it is to be consolidated, may or may not be a dense, coherent mass. The material in comminuted form gives best results if it is placed in a medium or vehicle which is preferably a liquid or at least is in a plastic state. The material placed in the vehicle may, in some cases, be dissolved in the latter while, in other instances, the vehicle should be of such nature that it will not dissolve the added material but merely hold it in suspension without reacting chemically therewith. The material added to the vehicle should be thoroughly distributed throughout the latter to obtain a homogeneous mixture. This mixture, in any desired concentration, is then applied to a material or body of any suitable nature, form or size, with which it is desired to unite the added material to produce a composite body. The combination thus obtained is then treated by any suitable means, such as mechanical working or by heating, to cause the applied material to permanently adhere to the other body and to cause the particles of the applied material to form a permanently coherent body. During this step in the process, the vehicle should, in most cases, be removed but, in other conceivable conditions, it may not be necessary to do so. In dealing with many materials it is necessary to give this treatment in an inert environment to avoid a change in the nature of the materials dealt with. In some cases, the atmosphere in contact with the materials employed may be an inert gas while the treatment of other materials requires the operations to be carried out in a vacuum and in still other instances an exceedingly high vacuum such, for example, as that obtained in a high-vacuum X-ray tube will give the best results.

Since it has been stated that one of the objects of this invention is the provision of a process for producing a composite body consisting, in part at least, of a metal of comparatively high electron emissivity, it will be shown in sufficient detail how such a body may be produced. Thorium will be selected as a metal representative of the class of metals possessing high electron emissivity and also as a member of the group of refractory metals. It is, moreover, a representative of that class of metals whose oxides are not reducible by hydrogen and of which class zirconium, uranium, beryllium, etc. are also members. Such metals, we have found, are particularly advantageous for increasing the efficiency and maintaining the candle power

of incandescent electric lamps, as explained above.

Molybdenum will be assumed as the base material to which the thorium is to be united. Thorium, in a powdered condition and in any desired quantity, may be mixed with a vehicle consisting of a solution of nitro cellulose in amyl acetate until a homogeneous mixture results. This mixture is then applied to a body of molybdenum which may, for example, be of wire form, by passing the molybdenum wire through the mixture. The quantity of thorium deposited on the wire will obviously depend on such factors as the concentration of thorium in the mixture, the rate at which the wire is passed through it, and the nature of the vehicle. The coated wire is then preferably placed in an air-tight vessel and connected therein to electrical conducting terminals sealed into the vessel. The latter is subsequently exhausted to a very high degree of vacuum by means of a pump which is preferably of the diffusion type. While maintaining the high vacuum in the vessel, electric current is passed through the coated wire which is thus heated to a temperature sufficiently high to remove the vehicle by volatilization and to cause the particles of thorium to be agglomerated and form a dense, coherent mass permanently adherent to the molybdenum base. The electric current passing through the wire is then cut out and the wire is allowed to cool before it is withdrawn from the vessel.

It is to be understood that the composite bodies produced according to the present invention may consist of two or more consolidated materials and that each component part may consist of mixtures or alloys. For example, a mixture of powdered thorium and powdered aluminum may be applied to a wire of molybdenum or tungsten, and the aluminum will then serve as a clean-up agent, preserving the thorium unoxidized to act as an electron emitter. Other variations in the products and process of this invention will be apparent to those skilled in the art but we desire it to be understood that such are part of our invention as set forth in the appended claims.

What is claimed is:

1. A composite refractory metal body, comprising molybdenum as a base and thorium consolidated therewith, said thorium having been first applied thereto as a suspension in a binder liquid and subsequently permanently consolidated thereto by heat in an inert environment.

2. A composite body comprising a base of molybdenum having thorium consolidated thereto, said thorium having been first applied to said base as a suspension in a binder liquid and subsequently permanently consoli-

dated thereto by heat in an inert environment.

3. Electron emission material comprising a base of molybdenum coated with thorium in a coherent and homogeneous state.

4. Electron-emission material comprising a filamentary body with a coating thereon of a powdered mixture of one of the group of metals consisting of thorium, zirconium, uranium, titanium and vanadium as the active electron-emitter and one of the group of metals consisting of aluminum, magnesium, chromium and the rare earth metals as a clean-up agent and protector of the active electron-emitter.

5. As an article of manufacture, a composite metallic body comprised of a molybdenum metal base member surfaced at least in part with an adherent, coherent, homogeneous coating of thorium.

In testimony whereof, we have hereunto subscribed our names this 30 day of July, 1921.

JOHN WESLEY MARDEN.

25 HARVEY CLAYTON RENTSCHLER.

30

35

40

45

50

55

60

65